

# United States Patent Office

3,169,869

Patented Feb. 16, 1965

1

3,169,869

## DIAZOTYPE MATERIAL

Andreas Joseph Johannes Hendrickx, Venlo, Limburg, Netherlands, assignor to Chemische Fabriek L. van der Grinten N.V., Venlo, Limburg, Netherlands, a corporation of the Netherlands

No Drawing. Filed May 26, 1959, Ser. No. 815,781  
Claims priority, application Netherlands, June 4, 1958,

228,409

9 Claims. (Cl. 96—91)

The invention relates to diazotype material of the so-called one-component type (which consists of sheet material carrying a layer of a light-sensitive diazo compound) and of the so-called two-component type (which consists of sheet material carrying a layer comprising both a light-sensitive diazo compound and an azo coupling component).

In Belgian patent specification No. 564,343 diazotype material is described which contains a diazo compound of the general Formula I:



in which X represents an anion, R<sub>1</sub> an alkyl group having at most 4 carbon atoms, R<sub>2</sub> an alkyl group having at most 4 carbon atoms or an aralkyl group having at most 7 carbon atoms, and R<sub>3</sub> an alkyl group having at most 4 carbon atoms.

Diazo compounds of this type are very sensitive to the light of the mercury-vapour lamps commonly employed in the diazotype process, both of high-pressure lamps and of low-pressure lamps, and both of the actinically fluorescent and of the non-fluorescent lamps.

Diazotype material sensitized with such a diazo compound is very suitable for the visual observation of the end point of the exposure in the process of copying by the light of actinically fluorescent mercury-vapour lamps.

The diazo compounds of this type having larger alkyl groups, such as n-butyl, and those having aralkyl groups, such as benzyl, often precipitate from their aqueous solutions if the customary quantity of the stabilizer naphthalene 1,3,6-trisulphonic acid (which is practically indispensable in light-sensitive diazotype layers) or one of its salts is added to them. In practice, water is preferably used as solvent for the manufacture of sensitizing liquids for diazotype materials. Hence, if normal sensitizing liquids are employed, it is not possible to use the normal quantities of this stabilizer in intimate admixture with the said diazo compounds though adequate quantities are necessary to obtain the stabilizing effect.

Sometimes the formation of precipitates can be prevented by addition of a large excess of stabilizer, but this involves other drawbacks. The solution then penetrates too far into the support of the diazotype material to which it is applied, especially if this support is paper; the diazotype material manufactured with it develops less satisfactorily, especially in the so-called semi-wet development process, in which a thin layer of developing liquid of, for example, 8 g./m.<sup>2</sup> is applied on the imagewise exposed diazotype material; the copies on the diazotype material manufactured with it often show an exposed background with a yellowish colour and sometimes serious discolouration upon exposure to the light.

The formation of precipitates can sometimes also be prevented, or precipitates already formed can be dissolved again, by dilution of the diazo solution, but diazotype material manufactured with such a diluted diazo solution yields only very weak copies.

2

The formation of precipitates can sometimes also be prevented, or precipitates already formed can be dissolved, by considerably raising the temperature of the water or of the solution (for example to 60° C.), but this measure has a deleterious effect on the keeping qualities of the sensitizing liquid and on the quality of the diazotype material manufactured with it. In practice sensitizing liquids at room temperature or at an even lower temperature are preferably used. Small increases of temperature, for example to 30° C., may be permitted.

The diazo compounds of general Formula I having small alkyl groups, for example 1-diazo 4-dimethylamino 3-methoxy benzene and 1-diazo 4-dimethylamino 3-ethoxybenzene, do not, under normal conditions, give a precipitate with the said stabilizer, but they yield light-coloured azo-dyestuffs and their coupling activity is low. Consequently, in practice the compounds with larger alkyl groups or those with aralkyl groups are preferred. They yield darker azo-dyestuffs and they couple more actively, which is especially important for diazotype material intended for semi-wet development.

Many azo-dyestuffs formed by the coupling of several of the diazo compounds according to Belgian patent specification No. 564,343 with the azo components commonly used in the diazotype process, such as phloroglucinol, 2,3-dihydroxy naphthalene, 2,3-dihydroxy naphthalene 6-sulphonic acid, 2-hydroxy naphthalene 3,6-disulphonic acid and the like, change their colour when the pH decreases. The surface of diazotype copies may turn acid or more acid after the development, either locally, for example owing to spilling of acid liquids, or wholly, for example when the copies are kept in a moist atmosphere, in consequence of which the acid from the interior of the paper can diffuse to the surface. As is known, base-paper for the diazotype process often contains rather large quantities of acid, for example in the form of alum. In consequence of a resultant decrease of the pH the said azo-dyestuffs often show an undesirable change of colour.

The compound 1-diazo 4-dimethylamino 3-methoxy 6-chlorobenzene, just like the corresponding compound without a chloro substituent, does not give precipitates with naphthalene 1,3,6-trisulphonic acid or its salts during the manufacture of normal aqueous sensitizing solutions. However, its coupling activity is low and the azo dyestuffs derived from it are light-coloured.

According to the present invention there is provided diazotype material which contains a diazo compound of the general Formula II:



in which X is an anion, Y a fluorine or chlorine atom, and R<sub>4</sub>, R<sub>5</sub>, and R<sub>6</sub> are hydrocarbon radicals chosen from alkyl groups having at most 4 carbon atoms and aralkyl groups having at most 11 carbon atoms, and R<sub>4</sub>, R<sub>5</sub>, and R<sub>6</sub> contain together at least 6 and at most 17 carbon atoms.

The diazo compounds of this type couple more actively than the corresponding compounds without a fluoro or chloro substituent. Moreover, compared with 1-diazo 4-dimethylamino 3-methoxy 6-chlorobenzene, referred to above, they are more active, give darker coloured azo dyestuffs and when used in one-component diazotype material cause less trouble with "bleeding" of the image portions, in which the formation of azo dyestuffs takes place during the so-called semi-wet development with an aqueous developing liquid.

The said "bleeding" is inconvenient and is manifested in the less sharp delineation of the said image portions and the broadening, for example, of the lines.

As compared with the corresponding compounds without a fluoro or chloro substituent, it is found that, during the preparation of normal aqueous sensitizing solutions, the diazo compounds of general Formula II surprisingly form smaller amounts of precipitates with naphthalene 1,3,6-trisulphonic acid or its salts, many of them giving no precipitate at all.

In consequence, diazotype material according to the invention can be manufactured with a sufficiently high diazo content and with a normal content of naphthalene 1,3,6-trisulphonic acid or one of its salts, and then has better keeping qualities than diazotype material of which the light-sensitive layer contains a corresponding diazo compound without a fluoro or chloro substituent and does not contain the said stabilizer.

The compatibility with the said stabilizer is not the same for all compounds of general Formula II. According as, for example, the size of the substituents  $R_4$ ,  $R_5$  and  $R_6$  increases, the compatibility will decrease. Yet even the compounds with the largest substituents  $R_4$ ,  $R_5$ , and  $R_6$  are more compatible with the said stabilizer than the corresponding diazo compounds without a fluoro or chloro substituent. Hence, during the preparation of sensitizing liquids for diazotype material according to the invention with diazo compounds with large substituents  $R_4$ ,  $R_5$  and  $R_6$ , precipitation difficulties with the said stabilizer can be avoided more easily (for example, by a small increase of the temperature) than during the preparation of sensitizing liquids with corresponding diazo compounds without a fluoro or chloro substituent.

Accordingly as the total number of carbon atoms of the substituents  $R_4$ ,  $R_5$  and  $R_6$  increases, the solubility of the diazo compounds in aqueous sensitizing liquids generally decreases. The compounds in which  $R_4$ ,  $R_5$  and  $R_6$  contain together more than 17 carbon atoms and in which no special solubilizing substituents, such as sulphonate acid groups, are present are only slightly soluble therein.

The azo-dyestuff images formed in diazotype material according to the invention are more resistant to decrease of the pH than the corresponding azo-dyestuff images in corresponding diazotype material sensitized with corresponding diazo compounds without a fluoro or chloro substituent.

The colour of the azo-dyestuffs formed by development, with ammonia vapour, of two-component diazotype material according to the invention, containing the azo-dyestuff component 7'-hydroxy naphtho-1',2', 4,5-imidazole, is stronger and purer than that of the azo-dyestuffs formed by development, with ammonia vapour, of corresponding two-component diazotype material containing a corresponding diazo compound without a fluoro or chloro substituent.

The diazotype material according to the invention, just like that made with the aforesaid diazo compounds without a fluoro or chloro substituent, is very sensitive to the light of mercury-vapour lamps and also very suitable for the visual observation of the end point of the exposure in the process of copying by the light of actinically fluorescent mercury-vapour lamps.

Diazo compounds which can be used in diazotype material according to the invention are:

- 4-dimethylamino 3-isobutoxy 6-chlorobenzene diazonium chloride, zinc chloride double salt,
- 4-dimethylamino 3-naphthylmethoxy 6-chlorobenzene diazonium chloride, zinc chloride double salt,
- 4-diethylamino 3-ethoxy 6-chlorobenzene diazonium chloride, zinc chloride double salt,
- 4-N-ethyl N-n-butylamino 3-ethoxy 6-fluorobenzene diazonium chloride, stannic chloride double salt,

- 4-dibenzylamino 3-methoxy 6-chlorobenzene diazonium sulphate,
- 4-N-hydroxyethyl N-benzylamino 3-methoxy 6-chlorobenzene diazonium chloride, zinc chloride double salt,
- 4 - N - methyl N - 3',4' - dichlorobenzylamino 3-methoxy 6-chlorobenzene diazonium chloride, cadmium chloride double salt,
- 4-N- $\beta$ -chloroethyl N-benzylamino 3-methoxy 6-chlorobenzene diazonium-borofluoride,
- 4-N-isopropyl N-benzylamino 3-ethoxy 6-chlorobenzene diazonium chloride, zinc chloride double salt,
- 4-N-methyl N-naphthylmethylamino 3-ethoxy 6-chlorobenzene diazonium chloride, zinc chloride double salt.

The diazo compounds in which  $R_4$ ,  $R_5$  and  $R_6$  contain together at least 8 carbon atoms are particularly suitable for the manufacture of one-component diazotype material. This one-component diazotype material can be easily and completely developed according to the semi-wet process with a developing liquid containing phloroglucinol. The developed copies do not show "bleeding."

Of the last-mentioned group of diazo compounds, those in which  $R_4$  represents a benzyl group are very suitable for the manufacture of one-component diazotype material. Copies on this material can also be developed satisfactorily without bleeding according to the semi-wet process with a developing liquid containing phloroglucinol. Moreover, they show a very clear, exposed background.

The diazotype material according to the invention may of course contain mixtures of diazo compounds. Accordingly as those mixtures have a lower content of diazo compound as described above, the diazotype material manufactured with these mixtures will also possess the advantages described to a less extent.

The diazo compounds used in the diazotype material according to the invention may be prepared in several ways. The starting material may, for example, be p-chloro-phenol. After alkylation or aralkylation of the hydroxy group the substance is nitrated, the ortho-nitro p-chloro-phenol ether is collected and reduced, and the resulting amino group is aralkylated and/or alkylated. The o-dialkyl (or alkyl-aralkyl or diaralkyl) amino p-chloro-phenol ether obtained is subsequently provided, in the para position with respect to the amino group, with a nitroso group by treatment with nitrous acid, or it is nitrated or coupled to diazotized 2,5-dichloroaniline. The nitroso or nitro compound or the azo-dyestuff obtained is reduced to an amino compound and this amino compound is converted into a diazonium compound by treatment with nitrous acid. The diazonium compound can be collected as a double salt, for example, by precipitation with zinc chloride or sodium borofluoride.

With regard to the above-mentioned alkylation of the amino group it is remarked that  $R_4$  and  $R_5$  may be the same or different alkyl groups and that their carbon chains may or may not be branched.

The following examples will serve to illustrate the invention.

#### Example I

- 60 White base-paper of weight 80 g./m.<sup>2</sup> for the diazotype process is sensitized with a solution (at 18° C.) of:
  - 21.5 g. of 4-N-methyl N-benzylamino 3-methoxy 6-chlorobenzene diazonium chloride, zinc chloride double salt
  - 5 g. of tartaric acid
  - 20 g. of naphthalene 1,3,6-trisulphonic acid sodium salt
  - 0.8 g. of methyl cellulose
 in 1000 cm.<sup>3</sup> of water and dried.
- 70 The sensitized surface contains approximately 0.55 millimole of the diazo compound per m.<sup>2</sup>. The diazotype paper has good keeping qualities.
- 75 A sheet of the diazotype material is exposed in contact with a film positive of a line-drawing in an exposure ap-

paratus equipped with actinically fluorescent low-pressure mercury-vapour lamps, with the film positive between the light-source and the diazotype paper. Exposure is continued until in the portions corresponding to the transparent portions of the film positive all the diazo compound has bleached out. The progress of the bleaching of the yellow diazo compound can easily be observed visually, for example, from the direction of the lamp.

The latent diazotype copy thus obtained is developed by applying on its image surface a layer of approximately 8 g./m.<sup>2</sup> of the following developer:

31 g. of thiourea  
6.5 g. of phloroglucinol  
6.5 g. of resorcinol  
2 g. of isopropylnaphthalene sulphonic acid sodium salt  
5 g. of sorbitol  
15 g. of saccharose  
53 g. of potassium tetraborate (5 aq.)  
9 g. of potassium hydroxide

in 1000 cm.<sup>3</sup> of water.

Very soon after the application of the layer of developer the developed copy shows a strong dark brown positive azo-dyestuff image on a clear white background. The lines of the image do not show bleeding.

If instead of the above-mentioned diazo compound an equimolar quantity of the corresponding compound without a chloro substituent is used, a precipitate is formed in the sensitizing liquid. If the non-chlorinated diazo compound is used in the absence of naphthalene 1.3.6-trisulphonic acid, no precipitate is formed, but the keeping qualities of the diazotype material produced are considerably inferior to those of the material according to the example.

The diazo compound used according to this example is prepared as follows:

2-methoxy 5-chloroaniline is benzylated. The product thus formed, 2-methoxy 5-chloro N-benzyl aniline (boiling point 1.5mm. 175-185° C.), is methylated to 2-methoxy 5-chloro N-methyl N-benzyl aniline (boiling point 1.5mm. 200-210°; melting point 45-46° C.), and subsequently nitrated to 2-methoxy 4-nitro 5-chloro N-methyl N-benzyl aniline (orange-yellow crystals, melting point 114-115° C.). This compound is reduced and worked up into the diazo compound in the usual way.

#### Example II

White base-paper of weight 80 g./m.<sup>2</sup> for the diazotype process is sensitized with a solution (at 18° C.) of:

17.5 g. of 4-N-methyl N-benzylamino 3-methoxy 6-chlorobenzene diazonium chloride, zinc chloride double salt  
100 g. of tartaric acid  
30 g. of boric acid  
20 g. of 7'-hydroxy naphtho-1',2', 4.5-imidazole HCl-salt  
0.8 g. of methyl cellulose  
in 1000 cm.<sup>3</sup> of water and dried.

The sensitized surface contains approximately 0.45 millimole of the diazo compound per m.<sup>2</sup>. A sheet of the diazotype paper is exposed as in Example I.

The latent diazotype copy thus obtained is developed by exposing it for some tens of seconds to hot concentrated moist ammonia vapour. A strong bright red positive image on a clear white background is obtained.

If instead of the above-mentioned diazo compound an equimolar quantity of the corresponding compound without a chloro substituent is used, a copy with a less strong and a less bright brown-red image is obtained. When the last-mentioned copy is moistened with dilute phosphoric acid, which may happen in workshops working with mordant baths, the red-brown colour of the copy turns yellow. The bright red colour of the copy according to this example, however, only changes when it is moistened with a much more concentrated phosphoric acid.

#### Example III

White base-paper of weight 80 g./m.<sup>2</sup> for the diazotype process is sensitized with a solution (at 18° C.) of:

5 23 g. of 4-N-n-propyl N-benzylamino 3-methoxy 6-chlorobenzene diazonium chloride, zinc chloride double salt  
3 g. of tartaric acid  
1 g. of citric acid  
35 g. of naphthalene 1.3.6-trisulphonic acid sodium salt  
20 cm.<sup>3</sup> of polyvinyl acetate dispersion (Vinnapas H.60) in 1000 cm.<sup>3</sup> of water and dried.

The sensitized surface contains approximately 0.5 millimole of the diazo compound per m.<sup>2</sup>. The diazotype paper has good keeping qualities. A sheet of the diazotype paper is exposed as in Example I.

The latent diazotype copy thus obtained is developed by applying on its image surface a layer of approximately 9 g./m.<sup>2</sup> of the following developer:

20 40 g. of thiourea  
4 g. of phloroglucinol  
1 g. of resorcinol  
1.2 g. of 2-ethylhexyl sulphuric acid mono-ester as sodium salt (commercially available under the name of Tergitol 08)  
25 200 g. of tert. sodium citrate (5 aq.)  
2 g. of citric acid  
in 1000 cm.<sup>3</sup> of water.

30 The developing liquid has a pH of about 6. The developed copy shows a strong black positive image on a clear white background which does not show any appreciable bleeding.

If instead of the above-mentioned diazo compound an equimolar quantity of the corresponding compound without a chloro substituent is used, a precipitate is formed in the sensitizing liquid. If the non-chlorinated diazo compound is used in the absence of naphthalene 1.3.6-trisulphonic acid, no precipitate is formed, but the keeping qualities of the diazotype material produced are considerably inferior to those of the material according to this example.

If the non-chlorinated diazo compound is used in the presence of an excess of naphthalene 1.3.6-trisulphonic acid, for example 60 g. instead of 35 g., again no precipitate will be formed, but the sensitizing liquid then obtained penetrates far into the paper, the diazotype paper manufactured with it develops more slowly and less completely, and copies on this diazotype paper show an exposed background with a yellowish colour.

The diazo compound used according to this example is prepared as follows:

2-methoxy 5-chloroaniline is converted with p-toluene sulphonyl chloride into the 2-methoxy 5-chloro p-tosyl anilide (melting point 143° C.). This compound is treated with n-propyl bromide and the 2-methoxy 5-chloro N-n-propyl N-p-tosyl anilide thus formed is hydrolyzed to 2-methoxy 5-chloro N-n-propyl aniline (boiling point<sub>15mm.</sub> 150-154° C.). This compound is benzylated and the 2-methoxy 5-chloro N-n-propyl N-benzyl aniline thus obtained (boiling point<sub>2mm.</sub> 186-190° C.) is converted into the desired diazo compound by nitrosation, reduction, and diazotization.

#### Example IV

65 65 Cellulose acetate film of 110 g./m.<sup>2</sup>, superficially hydrolyzed on one side, is sensitized by immersing it in a solution (at 18° C.) of:

70 21 g. of 4-di-n-propylamino 3-methoxy 6-chlorobenzene diazonium chloride, zinc chloride double salt  
5 g. of tartaric acid  
2 g. of boric acid  
20 g. of naphthalene 1.3.6-trisulphonic acid sodium salt  
75 250 cm.<sup>3</sup> of ethanol

in 750 cm.<sup>3</sup> of water, squeezing off the excess of liquid, and drying the film.

The sensitized surface contains approximately 0.8 millimole of the diazo compound per m.<sup>2</sup>. The diazotype film has good keeping qualities.

A sheet of the diazotype film, pressed between a reflectographic screen and a non-transparent original, for example a page from a book, is exposed to the light of a high-pressure mercury-vapour lamp, with the screen turned towards the light-source and in contact with the sensitized surface of the film.

After the termination of the exposure the latent reflex copy is developed by applying on its image surface a layer of approximately 9 g./m.<sup>2</sup> of the following developer:

10 g. of thiourea  
10 g. of borax  
17 g. of 3-methoxy sodium phenolate  
4 g. of isopropyl naphthalene sulphonic acid as sodium salt  
2 g. of ethylene diamine tetra-acetic acid sodium salt  
35 g. of sodium carbonate

in 1000 cm.<sup>3</sup> of water.

The developed copy shows a strong brown image, the lines of which do not show bleeding. The brown azo-dyestuff has good absorption for ultra-violet light. The copy therefore is very suitable as daughter original for the production of further copies on diazotype paper.

If instead of the above-mentioned diazo compound an equimolar quantity of the corresponding compound without a chloro substituent is used, the diazotype film manufactured with it develops more slowly and less completely. The azo-dyestuff of the copies on such a film has less absorption for ultra-violet light and the copies are less suitable as daughter originals than the copies according to this example. The azo-dyestuff image of the copies according to this example is more resistant to the action of acid than that of the copies on diazotype film manufactured with a corresponding compound without a chloro substituent.

The diazo compound used according to this example is prepared as follows:

2-methoxy 5-chloroaniline is converted with n-propyl bromide into 2-methoxy 5-chloro N,N-di-n-propyl aniline (boiling point<sub>15mm.</sub> 151–152° C.) Upon nitration, 2-methoxy 4-nitro 5-chloro N,N-di-n-propyl aniline (yellow needles, melting point 82° C.) is formed, which is converted into the desired diazo compound by reduction and diazotization.

#### Example V

White base-paper of weight 80 g./m.<sup>2</sup> for the diazotype process, with an acid content such that it has a pH of 4.1 when moistened with water, is sensitized with a solution (at 18° C.) of:

21 g. of 4-di-n.propylamino 3-methoxy 6-chlorobenzene diazonium chloride, zinc chloride double salt  
40 g. of tartaric acid  
10 g. of boric acid  
20 g. of naphthalene 1.3.6-trisulphonic acid sodium salt  
20 g. of 2-naphthol 3.6-disulphonic acid sodium salt  
0.8 g. of methylcellulose

in 1000 cm.<sup>3</sup> of water and dried.

The sensitized surface contains approximately 0.55 millimole of the diazo compound per m.<sup>2</sup>. The diazotype paper has good keeping qualities. A sheet of the diazotype paper is exposed as in Example I.

The latent diazotype copy thus obtained is developed by exposing it for some tens of seconds to hot concentrated moist ammonia vapour. A strong violet positive image is obtained, the colour of which does not change when the copies are kept in a moist atmosphere.

If instead of the above-mentioned diazo compound an equimolar quantity of the corresponding compound without a chloro substituent is used, again a copy with a violet image is obtained, the colour of which, however, changes considerably when the copy is kept in a moist atmosphere.

#### Example VI

White base-paper of weight 80 g./m.<sup>2</sup> for the diazotype process is sensitized with a solution (at 18° C.) of:

21 g. of 4-N-methyl N-benzylamino 3-methoxy 6-fluorobenzene diazonium chloride, zinc chloride double salt  
5 g. of tartaric acid  
15 2 g. of boric acid  
20 g. of naphthalene 1.3.6-trisulphonic acid sodium salt  
30 cm.<sup>3</sup> of polyvinyl acetate dispersion (Vinnapas H.60)

in 1000 cm.<sup>3</sup> of water and dried.

The sensitized surface contains approximately 0.5 millimole of the diazo compound per m.<sup>2</sup>. The diazotype paper has good keeping qualities.

A sheet of the diazotype paper is exposed and developed as in Example I. The developed copy shows a strong dark-brown positive image on a clear white background. The lines of the image do not show bleeding. Upon moistening with an acid liquid with pH 2, the azo-dyestuff does not show a change of colour.

If instead of the above-mentioned diazo compound an equimolar quantity of the corresponding compound without a fluoro substituent is used, a precipitate is formed in the sensitizing liquid.

If the non-fluorinated diazo compound is used in the absence of naphthalene 1.3.6-trisulphonic acid, no precipitate is formed, but the keeping qualities of the diazotype material manufactured with this sensitizing liquid are considerably inferior to those of the material according to this example.

The azo-dyestuff image of the copies on diazotype material manufactured with the corresponding compound without a fluoro substituent upon moistening with the above-mentioned acid liquid shows a change of colour.

The diazo compound used according to this example is prepared as follows:

45 O-nitro p-fluoro-anisole is reduced. The 2-methoxy 5-fluoroaniline thus obtained is tosylated. The product formed, 2-methoxy 5-fluoro N-tosyl aniline (melting point 125–126° C.), is methylated to 2-methoxy 5-fluoro N-methyl N-tosyl anilide (melting point 125° C.), and subsequently hydrolyzed to 2-methoxy 5-fluoro N-methyl aniline. This product is benzylated to 2-methoxy 5-fluoro N-methyl N-benzyl aniline (boiling point<sub>15mm.</sub> 185–190° C.) and subsequently nitrated to 2-methoxy 4-nitro 5-fluoro N-methyl N-benzyl aniline (melting point 60–61° C.).  
55 This compound is reduced and worked up into the diazo compound in the usual way.

#### Example VII

60 Natural transparent paper of weight 70 g./m.<sup>2</sup> for the diazotype process is sensitized with a solution (at 18° C.) of:

22 g. of 4-dimethylamino 3-benzylxy 6-chloro-benzene diazonium chloride, zinc chloride double salt  
10 g. of citric acid  
15 g. of naphthalene 1.3.6-trisulphonic acid sodium salt  
20 cm.<sup>3</sup> of polyvinyl acetate dispersion (Vinnapas H.60)

in 1000 cm.<sup>3</sup> of water and dried.

The sensitized surface contains approximately 0.5 millimole of the diazo compound per m.<sup>2</sup>. The diazotype paper has good keeping qualities.

A sheet of the diazotype paper is exposed as in Example I. The latent diazotype copy thus obtained is developed

by applying on its image surface a layer of approximately 8 g./m.<sup>2</sup> of the following developer:

26 g. of thiourea  
6.5 g. of phloroglucinol  
6.5 g. of resorcinol  
2 g. of ethylene diamine tetra-acetic acid sodium salt  
1.5 g. of dibutyl naphthalene sulphonic acid sodium salt, commercially available under the name of Sorbit P  
32 g. of sodium carbonate

in 1000 cm.<sup>3</sup> of water.

The developed copy shows a strong dark-brown positive image, the lines of which do not show bleeding. It is suitable as a daughter original for the production of further copies on diazotype paper.

If instead of the above-mentioned diazo compound an equimolar quantity of the corresponding compound without a chloro substituent is used, a precipitate is formed in the sensitizing liquid. If the non-chlorinated diazo compound is used in the absence of naphthalene 1,3,6-trisulphonic acid, no precipitate is formed, but the keeping qualities of the diazotype material manufactured with this sensitizing liquid are considerably inferior to those of the material according to this example.

The diazo compound used according to this example is 25 prepared as follows:

2-nitro 4-chlorophenol is converted with benzyl chloride into 2-nitro 4-chlorophenylbenzyl ether (melting point 85-86° C., yellow crystals). This compound is reduced to 2-benzyloxy 5-chloroaniline (melting point 60° C.) and subsequently methylated to 2-benzyloxy 5-chloro N,N-dimethyl aniline (melting point 40° C.). Upon nitration, 2-benzyloxy 4-nitro 5-chloro N,N-dimethyl aniline (red leaflets, melting point 107° C.) is formed. This compound is reduced and worked up into the diazo compound 35 in the usual way.

I claim:

1. Diazotype material comprising a sheet material carrying a light-sensitive layer containing a diazo compound of the general formula



in which X is an anion, Y is an atom selected from the class consisting of fluorine and chlorine atoms, and R<sub>4</sub>, R<sub>5</sub> and R<sub>6</sub> are groups selected from the class consisting of alkyl groups having at most 4 carbon atoms and aralkyl groups having at most 11 carbon atoms, and R<sub>4</sub>, R<sub>5</sub> and R<sub>6</sub> contain together at least 6 and at most 17 carbon atoms.

2. One-component diazotype material according to claim 1, wherein, in the said diazo compound R<sub>4</sub>, R<sub>5</sub> and R<sub>6</sub> contain together at least 8 and at most 17 carbon atoms and wherein the said layer contains no azo coupling component.

3. One-component diazotype material according to claim 2, wherein, in the said diazo compound R<sub>4</sub> represents a benzyl group.

4. A diazotype material comprising a sheet-like support carrying a light-sensitive composition containing a diazo-

nium salt of 4-N - methyl N - benzylamino 3 - methoxy 6-chlorobenzene.

5. A diazotype material comprising a sheet-like support carrying a light-sensitive composition containing a diazonium salt of 4-N-methyl N - benzylamino 3 - methoxy 6-chlorobenzene.

6. A diazotype material comprising a sheet-like support carrying a light-sensitive composition containing a diazonium salt of 4-di-n-propyl-amino 3-methoxy 6-chlorobenzene.

10 7. A diazotype material comprising a sheet-like support carrying a light-sensitive composition containing a diazonium salt of 4-N-methyl N - benzylamino 3 - methoxy 6-fluorobenzene.

15 8. A diazotype material comprising a sheet-like support carrying a light-sensitive composition containing a diazonium salt of 4-dimethyl-amino 3-benzyloxy 6-chlorobenzene.

20 9. One-component diazotype material comprising a sheet material carrying a light-sensitive layer containing as a stabilizer a compound selected from the class consisting of naphthalene 1,3,6-trisulfonic acid and salts thereof, together with a diazo compound of the formula



30 in which X is an anion, Y is an atom selected from the class consisting of fluorine and chlorine atoms, and R<sub>4</sub>, R<sub>5</sub> and R<sub>6</sub> are groups selected from the class consisting of alkyl groups having at most 4 carbon atoms and aralkyl groups having at most 11 carbon atoms, and R<sub>4</sub>, R<sub>5</sub> and R<sub>6</sub> contain together at least 6 and at most 17 carbon atoms.

#### References Cited by the Examiner

##### UNITED STATES PATENTS

|    |           |       |                       |         |
|----|-----------|-------|-----------------------|---------|
| 40 | 2,037,542 | 4/36  | Schmidt et al. -----  | 96-91   |
|    | 2,113,944 | 4/38  | Leuch.                |         |
|    | 2,405,523 | 8/46  | Sease et al. -----    | 96-75   |
|    | 2,537,097 | 1/51  | Slifkin -----         | 96-75   |
|    | 2,551,133 | 5/51  | Jennings et al. ----- | 96-75   |
|    | 2,593,911 | 4/52  | Neumann -----         | 96-91   |
|    | 2,657,141 | 10/53 | Kessels -----         | 96-49   |
|    | 2,792,303 | 5/57  | Sanders et al. -----  | 96-49   |
|    | 2,822,272 | 2/58  | Kosalek et al.        |         |
|    | 2,937,085 | 5/60  | Seven et al. -----    | 96-75 X |

##### FOREIGN PATENTS

|         |      |                |
|---------|------|----------------|
| 643,309 | 9/50 | Great Britain. |
|---------|------|----------------|

##### OTHER REFERENCES

Venkataraman: Synthetic Dyes, vol. I, 1952, page 413.  
Saunders: The Aromatic Diazo Compounds (1949), pages 359-361.

Organic Chemistry, College Outline Series, by Degering, Barnes & Noble, N.Y., 1951, page 250.

NORMAN G. TORCHIN, Primary Examiner.

CHARLES B. PARKER, MILTON STERMAN, PHILIP E. MANGAN, ABRAHAM H. WINKELSTEIN,  
Examiners.

UNITED STATES PATENT OFFICE  
CERTIFICATE OF CORRECTION

Patent No. 3,169,869

February 16, 1965

Andreas Joseph Johannes Hendrickx

It is hereby certified that error appears in the above numbered patent requiring correction and that the said Letters Patent should read as corrected below.

Column 10, lines 5 and 6, strike out "4-N-methyl  
N-benzylamino 3-methoxy 6-chlorobenzene" read -- 4-N-n.propyl  
N-benzylamino 3-methoxy 6-chlorobenzene --.

Signed and sealed this 27th day of July 1965.

(SEAL)

Attest:

ERNEST W. SWIDER  
Attesting Officer

EDWARD J. BRENNER  
Commissioner of Patents